

H. JONES.  
METHOD OF FORMING BRAKE SHOES  
APPLICATION FILED JAN. 23, 1915.

1,167,826.

Patented Jan. 11, 1916.

Fig.1.



Fig. 2.



Fig. 3.



Fig. 4.



Fig. 5.



INVENTOR  
Harry Jones.

BY *George Cook*  
ATTORNEYS

*John Cook*  
*A. V. Walsh*

# UNITED STATES PATENT OFFICE.

HARRY JONES, OF SUFFERN, NEW YORK, ASSIGNOR TO AMERICAN BRAKE SHOE & FOUNDRY COMPANY, OF MAHWAH, NEW JERSEY, A CORPORATION OF NEW JERSEY.

## METHOD OF FORMING BRAKE-SHOES.

1,167,826.

Specification of Letters Patent. Patented Jan. 11, 1916.

Application filed January 23, 1915. Serial No. 3,875.

*To all whom it may concern:*

Be it known that I, HARRY JONES, a citizen of the United States, and a resident of Suffern, in the county of Rockland and 5 State of New York, have made and invented certain new and useful Improvements in Methods of Forming Brake-Shoes, of which the following is a specification.

This invention relates to a method for 10 making brake shoes.

The present invention comprehends the formation of a porous and lubricating coating upon a wire netting, or other insert of reticulated metal, which is subsequently inserted within a mold and the body of a 15 brake shoe cast therearound, the insert being so positioned, and of such dimensions, that it extends beyond the end, or ends, of the shoe body and is adapted to absorb a 20 suitable oil, which, commingling with the lubricating coating, materially increases the efficiency thereof.

A further object is to provide a method 25 whereby an oily and plastic insert may be directly embedded within a cast metal shoe, the end being attained by forming a porous, absorbent and lubricating coating upon the 30 insert and embedding the same directly within the metal of the shoe body, and subsequently inserting one of the exposed ends 35 of the said absorbent coating within a suitable oil, such as linseed or china wood, which, due to capillary action, flows throughout the entire coating, and commingling 40 with the ingredients thereof, renders the same plastic and cohesive, thus providing a noiseless and efficiently operating brake shoe.

A further object is to provide a method 45 for coating an insert for shoes, which, although formed of a lubricating substance, will be of a porous texture or nature, capable of lubricating the shoe, and further adapted to absorb an oil, rendering the 50 insert cohesive and plastic, insuring the successful operation thereof, all of which properties are not in any way injured by contact with the molten metal of the shoe as it is cast therearound.

55 Other objects and advantages of the method will appear as the description proceeds, wherein it is to be understood that changes in the precise procedure can be made within the scope of what is claimed

without departing from the spirit of the 55 invention.

As illustrating the manner in which the process is carried out, Figure 1 is a view in plan of the insert, in the form of a wire netting previous to its repeated immersion 60 within a mixture of graphite and sodium silicate; Fig. 2 is a similar view after the wire has been immersed within the mixture and after it has been subjected to a high 65 temperature, whereby it is rigidly baked to 70 the wire in the form of a porous, absorbent coating; Fig. 3 illustrates the brake shoe with the insert therein, extending therebeyond, and immersed within a suitable vessel containing oil, whereby the oil is absorbed and passes throughout the porous 75 coating so as to render the same cohesive and plastic; Fig. 4 is a view in side elevation, with portions thereof removed, of the completed brake shoe; Fig. 5 is a cross-sectional view taken on the line 5—5 of Fig. 4.

Referring specifically to the several figures, wherein similar reference numerals 80 designate corresponding parts throughout, 85 an insert 10, preferably formed of wire, expanded metal, open-work or reticulated metal, is cut to size so as to fit within a brake shoe mold, and of sufficient length to project beyond the end or ends of the shoe 90 which is to be cast therearound. The insert 10 is repeatedly dipped into a mixture of substantially equal parts, by volume, of sodium silicate and graphite, the same being allowed to dry after each dipping so 95 that a coating 11 may be built up of any desired thickness. The wire and coating is then subjected to a heat approximating 1200° F. whereby the water of crystallization of the sodium silicate will be driven off, 100 and the entire mass baked together so as to form a porous covering, which possesses sufficient rigidity and strength to withstand the action of the molten metal of the brake shoe as the same is cast therearound; the 105 coating, having been previously subjected to a high temperature, is not materially affected by the molten metal.

By the foregoing procedure, a brake shoe 12 is formed, having therein, either one or 105 more, inserts consisting of a plurality of connected and interlaced tubes of porous graphite, which are capable of lubricating

the wearing face of the shoe; but in order to prevent the graphite from flaking away when the shoe is in service, the exposed end of the insert is immersed in a vessel of oil, as illustrated in Fig. 3, whereby the oil will be absorbed by the porous coating or tubes and flows therethrough to mix or commingle with the various ingredients. The oil renders the insert cohesive and plastic, preventing the flaking away of the graphite and successfully eliminating all squeaking or noises incident to the application of the brake shoe to the wheel.

The oil, which may be linseed, china wood, or other suitable one, or mixture of oils, flows through the tubes of graphite due to the porosity thereof and commingles with and becomes a part of the lubricating tubes or coatings of the metal insert, which latter acts as supporting web or structure for the support of the tubes during the process of formation of the shoe and lubricating insert. The protruding end of the insert is then cut away, and the completed shoe has embedded therein a cohesive and plastic insert possessing lubricating qualities which will prevent the chattering and noise of the shoe without materially interfering with the proper braking properties thereof.

As a matter of fact, not only does the lubricating compound not interfere with the braking properties or qualities of the shoe, but actually enhances the same. It will be understood that in the manufacture of brake shoes, the harder the iron employed, the more lasting the shoe is in service. These lasting qualities are imparted to the shoe by constructing it of what is generally termed "white" or "hard" iron, that is, a metal wherein there is little or no graphitic or free carbon, the carbon being all, or for the most part, combined with the metal. In the shoe constructed as above described, the graphite is added to the shoe while in service, that is, added to the wearing surface thereof, and lends to the shoe the lubricant which the shoe would naturally have when made of the softer metal or gray iron, and in which instance the shoe is possessed of greater frictional qualities, due to the free or

graphitic carbon, the result being that while by my invention it is possible to use a white or hard iron to secure the lasting qualities of the shoe, yet the latter has imparted thereto the frictional qualities of a gray iron, due to the graphite added thereto in its free state.

What I claim is:

1. The method of forming brake shoes consisting in forming a coating, including graphite, upon an insert of metal, casting the body of a brake shoe therearound, and supplying a liquid oil to the said coating. 60
2. The method of forming brake shoes consisting in casting a shoe body around an insert including a porous mixture of graphite, positioning the said insert so as to protrude beyond the body of the shoe and immersing the protruding end of said insert into a bath of oil. 65
3. The method of forming brake shoes consisting in forming a plurality of interlaced or connected tubes of a porous mixture including graphite, casting the metal body of a shoe therearound, and supplying an oil 75 to the said porous tubes for the absorption thereof and rendering the said tubes capable of lubricating the shoe. 70
4. The method of forming brake shoes consisting in forming a plurality of interlaced or connected tubes of graphite and sodium silicate, casting a shoe body therearound, and supplying an oil to said porous tubes for the absorption of the former, thereby rendering said tubes capable of 85 lubricating the shoe. 80

5. The method of forming brake shoes consisting in coating reticulated metal with a porous mixture including graphite, casting a shoe body therearound, and supplying 90 oil to said porous coating.

Signed at New York, borough of Manhattan, in the county of New York and State of New York, this 12th day of January, A. D. 1915.

HARRY JONES.

Witnesses:

MARY B. JUSTICE,  
ANNA V. WALSH.